

Nov. 3, 1942.

H. A. LOMAX

2,300,792

MANUFACTURE OF ROLLS

Filed Nov. 10, 1939

2 Sheets-Sheet 1

Fig. 1



INVENTOR.

Harold A. Lomax  
BY Brown, Critchlow & Flick  
his ATTORNEYS.

Nov. 3, 1942.

H. A. LOMAX

2,300,792

MANUFACTURE OF ROLLS

Filed Nov. 10, 1939

2 Sheets-Sheet 2



Fig. 2.-1600°F.



Fig. 3.-1700°F.



Fig. 4.-1800°F.



Fig. 5.-2000 F.

INVENTOR  
Harold A. Lomax  
BY Brown, Coddow & Fleiss  
his ATTORNEYS.

## UNITED STATES PATENT OFFICE

2,300,792

## MANUFACTURE OF ROLLS

Harold A. Lomax, Wyomissing, Pa.

Application November 10, 1939, Serial No. 303,835

7 Claims. (Cl. 148—21.5)

This invention relates to rolls for use in rolling metal, more particularly to alloy steel rolls, especially for use in rolling hot steel.

A particular disadvantage of both cast iron and alloy steel rolls made heretofore is their tendency to fire crack or check. These surface defects may be, and commonly are, of appreciable size, both as to width and depth, and their occurrence necessitates resurfacing, by grinding or turning, of the roll to remove them because if not removed they impair the surface finish of the rolled metal. The occurrence of such surface defects in the rolls thus increases rolling costs undesirably, not only due to the cost of grinding, but also because of the reduction in roll diameter consequent upon removal of deep checks or frequent resurfacing.

A primary object of the invention is to provide a heat treatment for cast alloy steel rolls to confer resistance to fire cracking or checking superior to those of ordinary steel rolls.

Another object is to provide a heat treatment for cast alloy steel rolls which confers superior resistance to fire cracking and checking and in the practice of which the hardness produced may be varied according to need as well as to produce rolls of greater hardness than ordinarily developed heretofore in alloy steel rolls.

It is also an object of this invention to provide alloy steel rolls of simple and relatively inexpensive composition, which embody as a primary advantage high resistance to checking and fire cracking that is produced by a simple heat treatment, and which possess suitable hardness together with other desirable physical and mechanical properties, such as strength and shock resistance, adequate for use in rolling metal, particularly in hot rolling of steel.

Other objects of the invention will appear from the following description.

The invention will be described with reference to the accompanying drawings in which Fig. 1 is a graph showing the hardness of a roll steel alloy produced by cooling at different rates from different temperatures, and Figs. 2 to 5 photomicrographs illustrative of the microstructures produced by some of the heat treatments of Fig. 1.

The invention is predicated upon my discovery that improved resistance to fire cracking and checking of alloy steel rolls may be developed by their heat treatment in a particular manner, and that especially superior results are had by such heat treatment of rolls made from a particular type of alloy steel.

In accordance with the invention the alloy steel rolls are subjected to a heat treatment, or annealing, in which they are heated to substantially above the critical temperature, most suitably to at least about 1700° F., which is considerably above the critical temperature of the roll alloy steels. For many purposes a single heat treatment of this character suffices both to confer the improved resistance to fire cracking and checking and also to prepare the rolls for use. But where they are subjected to other heat treatments it is necessary either that this high temperature heat treatment be the final heating, or that subsequent heat treatment be confined to heating below the critical range.

As is customary in these heat treating operations, it is usually desirable that the rolls be held at the high temperature for a period of time.

This heat treatment in accordance with the invention produces a new grain structure in the roll of a type which roll makers and users have sought heretofore to avoid but which I believe is responsible for, or contributes largely to, the superior resistance to fire cracking of rolls made in accordance with the invention. That is, when this heat treatment is the final step, or at least the final treatment above the critical temperature, it causes recrystallization of the cast structure with production of grains surrounded by envelopes of cementite. The grains produced will be of increasing average size as the temperature of heat treatment increases, but in general will be smaller than those of the original cast structure, and as long as the temperature used is sufficiently above the critical range, they will possess the cementite envelopes referred to irrespective of the rate of cooling from temperature. This structure and the temperature necessary to produce it are illustrated in the drawings and discussed further hereinafter.

Where high hardness is desired the rolls are cooled at a relatively rapid rate from this heat treating temperature, and by variation of the heat treating temperature and the rate of cooling the hardness of the rolls may be varied within wide limits.

By appropriate selection of composition, heat treating temperature and cooling rate, therefore, there are produced rolls of satisfactory surface hardness which are highly resistant to fire cracking and checking, which phenomena have heretofore been a limiting factor in the life of such rolls. This improved resistance to fire cracking results from the application of the heat treat-

ment provided by the invention to alloy steel rolls, particularly the nickel-molybdenum steels described hereinafter and which when heat treated as described herein provide particularly improved resistance to checking and fire cracking. More in detail, the surfaces of rolls made in accordance with the invention do not fire or water crack with production of either large horizontal or circumferential fire cracks such as have heretofore been customarily encountered in other alloy steel rolls, such checking or crazing as may occur being narrow and shallow, and there being no particular tendency for these fine cracks to enlarge substantially. In consequence, when it is necessary to resurface the roll a perfectly satisfactory surface can be produced by removing as little as  $\frac{1}{16}$  to  $\frac{1}{8}$  of an inch from the roll surface, so that the rolls are capable of repeated resurfacing with attendant long life.

The invention may be described further with reference to alloy steels which have been found to be particularly adapted to the practice of the invention in producing rolls of exceptional resistance to fire checking and cracking, viz., nickel-molybdenum alloy steels. Preferably the steels are of low, or relatively low, content of chromium. More particularly, the steels preferably used in the practice of the invention contain carbon from about 0.75 to about 2.5 per cent, chromium up to about 0.5 per cent, manganese up to about 1.5 per cent, molybdenum more than about 0.2 per cent and desirably at least about 0.35 per cent, and substantial amounts of nickel, the remainder of the steel being effectively iron together with elements and impurities, such as phosphorus, silicon and sulfur, in amounts customary in such alloy steels or which do not depreciate the desirable properties of the steels, i. e., the remainder is substantially all iron. Inasmuch as the rolls are made from steel alloys it is preferred that the silicon content be relatively low, say not in excess of about 0.5 or 0.6 per cent. For many purposes it is preferred that the nickel content of the steel be about three to four times the content of silicon, and ordinarily the nickel content will be from about 1.5 to 2.5 per cent. For many purposes not over about 0.75 per cent of molybdenum suffices.

Rolls made from steels of the foregoing composition and heat treated in accordance with the invention will possess a surface hardness of from 46 to 58 Shore scleroscope, or about 320 to about 410 Brinell, depending upon the particular composition within the ranges stated and upon the details of the heat treatment. By changes in the ratio of the elements, for example nickel, silicon, chromium and carbon, the hardness of the roll surface, may be increased or decreased according to need so that it is possible in the practice of the invention to produce rolls which are particularly adapted to the various conditions encountered in the rolling of metal, for example steel.

For many purposes, and particularly for the manufacture of blooming mill rolls, it is preferred to cast the rolls from alloy steels containing from about 0.8 to 1.25 per cent of carbon, not over about 0.5 per cent of chromium, from about 0.8 to 1.2 per cent of manganese, from about 0.3 to 0.5 per cent of molybdenum, from about 1.6 to 1.8 per cent of nickel, and not over about 0.6 per cent of silicon. For most purposes the phosphorus and sulfur should be relatively low, say not over about 0.05 per cent each.

Through the use of nickel-molybdenum alloy steels of substantially the foregoing composition the rolls when heat treated in accordance with

5 the invention possess other physical properties which adapt them to use in rolling mills. For instance, they may possess a tensile strength of 110,000 pounds per square inch, so that they are extremely strong and of long life.

10 The particular temperature to which the rolls are heated and the precise rate at which they are cooled will depend, of course, upon the particular alloy steel composition used in making the roll, the temperature to which it is heated, and the 15 particular hardness or other mechanical properties desired. I have found by extended experience, however, that using an annealing temperature of 1700° F. cooling at an over-all rate of about 100° F. per hour to well below the critical range, say to 800° F., is productive of eminently 20 satisfactory results with rolls of the nickel-molybdenum steels described, and I believe this combination to be generally applicable to roll alloy 25 steels to produce the results which characterize the invention. The rolls may, of course, be cooled more rapidly, say at 300° F. per hour, provided that this does not cause them to be unsatisfactorily fragile. Heating at 1600° F. of these Ni-Mo steels does not produce a well-defined grain and 30 cementite envelope structure, and cooling at the slow rates that have been used heretofore in annealing rolls, e. g., 25° F. per hour, does not produce the high hardness that is possible through the practice of the invention. I now believe that 35 cooling rates of about 50° to about 300° F. per hour suffice generally in the practice of the invention.

The effects of the annealing temperatures and 40 cooling rates which characterize the invention may be exemplified further with reference to the drawings, which represent the results obtained with a roll steel alloy containing 1.08 per cent of carbon, 0.5 per cent of chromium, 0.89 per cent of manganese, 0.34 per cent of molybdenum, 1.58 per cent of nickel, and 0.34 per cent of silicon. Samples of this alloy were heated to various 45 temperatures (abscissae in Fig. 1) and cooled at different rates, and after they were at room temperature their hardness (ordinates in Fig. 1) was determined.

Reference to Fig. 1 shows that when the steel is cooled at the rate of about 100° F. per hour from 1600° F. the steel exhibits a Brinell hardness of about 285. However, with an annealing 50 temperature of 1700° F. and the same cooling rate the hardness was 321, which confers more satisfactory wear resistance. As shown also by Fig. 1, the same hardness may be had by cooling at 300° F. per hour from a lower temperature, i. e., about 55 1550° F.

The graphs show further that for a given rapid cooling rate the hardness increases with the annealing temperature, and that an increase in cooling rate results either in the production of 60 equivalent hardness from a lower annealing temperature, or increase in hardness for a given temperature. Finally, samples cooled at 25° F. per hour developed maximum hardness when cooled from 1700° F., and their hardness was much less than is attainable with more rapid cooling rates.

Figs. 2 to 5 are photomicrographs at 100 diameters magnification of some of the samples cooled at 100° F. per hour used in obtaining the data for Fig. 1. As appears therefrom, in this series of tests the original cast structure persists up to an annealing temperature of 1600° F. (Fig. 2). At 1700° F. (Fig. 3), however, the structure has undergone recrystallization with production of 70 grains that are smaller than in the original cast-

ing and are more or less completely enveloped at their boundaries by cementite. This is true also of annealing temperatures above 1700° F. (Figs. 4-5) although as the temperature increases the grain size increases also.

This may explain the substantially improved resistance to checking and fire cracking of rolls made in accordance with the invention. Thus, it will be noted that in the structures produced at and above 1700° F. the hard cementite at the grain boundary will tend to prevent transcrys-talline rupture in any grain from passing directly into an adjacent grain. Hence such a structure would tend to restrict the size and the enlargement of checks formed at the surface of the roll. On the other hand, it is reasonable to suppose that structures such as shown in Fig. 2 will not accomplish that result because once rupture starts at the surface it is relatively free to proceed unhampered and in a more or less straight line through the large and relatively soft grains to produce checks and cracks of large size and depth.

Although this presents a reasonable explanation of the results obtained in the practice of the invention, I do not limit myself to it because it is not known certainly whether the results are due primarily to the structural change just explained, or whether it is due primarily to the hardness developed by the heat treatment, coupled with other mechanical properties, or perhaps are due both to the structure and high hardness. For example, rolls cooled at 300° F. per hour from 1600° F. appear to possess the resistance to checking of rolls cooled at 100° F. per hour from 1700° F. although the grain structure of the former is not so well developed as in the latter. However, it is a fact that prior practice of cooling slowly from lower temperatures, say at 25° F. per hour from 1600° F., is not productive of the resistance to fire cracking which characterizes this invention. And the data given indicate the desirability of annealing at a temperature at which recrystallization occurs, and the beneficial effects of rapid cooling.

As an example, a 29 x 69½ inch blooming mill roll in accordance with the invention was heated to about 1700° F. in about twenty-eight hours and held at that temperature thirty hours, i. e., approximately one hour for each inch of roll diameter, which is satisfactory in most cases. It was then cooled to about 800° F. in ten hours.

Although in general the desirable practice is to subject the cast roll to a single anneal as described, tests indicate that it is not necessary to restrict the heat treatment in this manner, i. e., the essential thing seems to be that as a final step the roll be cooled from an elevated temperature as described, or, alternatively, that after being thus heated any further heat treatment be below the critical range.

According to the provisions of the patent statutes, I have explained the principle and mode of practicing my invention and have illustrated and described what I now consider to represent its best embodiment. However, I desire to have it understood that, within the scope of the appended claims, the invention may be practiced otherwise than as specifically illustrated and described.

I claim:

1. As a new article of manufacture, a roll formed from cast alloy steel, said roll being in heat treated condition, and having a recrystallized grain structure composed of grains smaller than those of the roll as cast and substantially surrounded by cementite envelopes, and being highly resistant to checking and fire cracking.
2. That method of heat treating a cast alloy steel rolling mill roll which comprises as the final heat treatment above the critical temperature heating the roll to a temperature substantially above the critical and then cooling it to a temperature below the critical range at a rate between about 25° and 300° F. per hour and thereby producing a structure of relatively coarse grains surrounded by cementite envelopes and rendering the roll resistant to fire cracking and checking.
3. A method according to claim 2, the roll being heated to at least about 1700° F. and being cooled at a rate of between about 50 and 300° F. per hour.
4. A method according to claim 2, the roll being made from an alloy containing about 0.75 to 2.5 per cent of carbon, from a small amount to not over about 0.5 per cent of chromium, from a small amount to not over about 1.5 per cent of manganese, from about 0.2 to 0.75 per cent of molybdenum, from a small amount to not over about 0.6 percent of silicon, nickel from about three to four times the content of silicon, and the remainder substantially all iron.
5. A method according to claim 2, the roll being made from an alloy containing about 0.75 to 2.5 per cent of carbon, from a small amount to not over about 0.5 per cent of chromium, from a small amount to not over about 1.5 per cent of manganese, from about 0.2 to 0.75 per cent of molybdenum, from a small amount to not over about 0.6 per cent of silicon, from about 1.5 to 2.5 per cent of nickel, and the remainder substantially all iron, and the roll being heated to at least about 1700° F. and being cooled at a rate between about 50° and 300° F. per hour.
6. A method according to claim 2, in which the roll is made from an alloy containing about 0.8 to 1.25 per cent of carbon, from a small amount to not over about 0.5 per cent of chromium, from about 0.8 to 1.2 per cent of manganese, from about 0.3 to 0.5 per cent of molybdenum, about 1.6 to 1.8 per cent of nickel, from a small amount to not over about 0.5 per cent of silicon, and the remainder substantially all iron.
7. As a new article of manufacture, a rolling mill roll formed from cast alloy steel containing about 0.75 to 2.5 per cent of carbon, from a small amount to not over about 0.5 per cent of chromium, from a small amount to not over about 1.5 per cent of manganese, about 0.2 to 0.75 per cent of molybdenum, about 1.5 to 2.5 per cent of nickel, from a small amount to 0.6 per cent of silicon, and the remainder substantially all iron, said roll having a structure composed of recrystallized grains that are surrounded by cementite envelopes and are relatively coarse but smaller than the grains of the roll as cast, and the roll being highly resistant to checking and fire cracking.